

W. J. WOOLDRIDGE,  
ANNEALING MAGNETIC MATERIAL,  
APPLICATION FILED DEC. 17, 1918.

1,331,889.

Patented Feb. 24, 1920.

Fig. 1.



Fig. 3.



Fig. 4.



Fig. 5.



Fig. 2.



Inventor:  
William J. Wooldridge,  
by *Albert H. Davis*  
His Attorney.

# UNITED STATES PATENT OFFICE.

WILLIAM J. WOOLDRIDGE, OF PITTSFIELD, MASSACHUSETTS, ASSIGNOR TO GENERAL ELECTRIC COMPANY, A CORPORATION OF NEW YORK.

## ANNEALING MAGNETIC MATERIAL.

1,331,889.

Specification of Letters Patent. Patented Feb. 24, 1920.

Application filed December 17, 1918. Serial No. 267,110.

To all whom it may concern:

Be it known that I, WILLIAM J. WOOLDRIDGE, a citizen of the United States, residing at Pittsfield, in the county of Berkshire, State of Massachusetts, have invented certain new and useful Improvements in Annealing Magnetic Materials, of which the following is a specification.

My invention has reference to improvements in the process of annealing magnetic material, mainly silicon steel in sheet form, and it consists in exposing and supporting the sheet material while subjected to the annealing temperature, in annealing pots or otherwise, in such manner as to give free access of heat radiation to and circulation of evolved gases over the material on all sides, whereby the sheets are annealed uniformly through their whole extent.

Magnetic sheet material has heretofore been annealed by placing the sheets in well known annealing pots, stacked flatwise one above the other and each in contact with the preceding and succeeding sheets and each under the pressure of the weight of the upper pile. In this manner all sheets are partially shielded from the direct heat radiation from the walls of the annealing pot, and the gases which are evolved from the sheets in the pot or enter the pot from the furnace cannot freely circulate over the faces of the material. The consequence is that the annealing effect is limited to more or less irregular portions near the edges of the sheets, while the more central portions are poorly, and in many cases not at all, annealed. By my invention this detrimental effect of the stacking of the sheets one on top of the other is avoided, and practically uniform and effective annealing all throughout the sheets is achieved. This result has heretofore been attained by assembling and maintaining the whole charge of sheets loosely face to face with small but sensible spaces between them, and resting edgewise on the floor of the annealing pot, and subjecting the pot to the requisite temperature. But while in this manner the sheets became well annealed, they buckled considerably when softened by the high temperature to which they had to be raised, under the pressure of the weight of each sheet upon its supporting edge. Moreover, the assembling of a great number of sheets which constitute the charge of a pot, in the manner in-

dictated, and the maintenance of the assemblage, has been found to be uncertain, difficult and time consuming, so that in commercial practice the advantages of the otherwise correct process could not be realized. My invention is an improvement upon the process just described, whereby the disadvantages pointed out are avoided and an efficient commercial practice is secured.

In the accompanying drawing the old practice of piling the sheets flatwise on top of each other, its result, and the present inventions are illustrated as follows: Figure 1 is a vertical section of an annealing pot with the material to be annealed piled up flatwise in the old conventional manner; Fig. 2 is a face view of one sheet of a stack subjected to the old practice, showing by appropriate shading the resulting imperfect annealing; Fig. 3 is a vertical section of an annealing pot with bundles of sheets arranged in the same in accordance with one of the practices of my invention; Fig. 4 is a like section at right angles to that shown in Fig. 3 of an annealing pot with bundles of sheets arranged in the same in accordance with another practice of my invention, and Fig. 5 is a perspective view of a bundle of sheets, which in the practice of my invention is a unit corresponding to the single sheets in the old processes.

Referring now to Fig. 1, the ordinary annealing pot 10 with its legs 11 and its cover 12, has the sheets 13, stacked up, as indicated, flatwise one on top of the other with no appreciable spaces between them, so that each sheet covers every preceding one and is in turn covered by the succeeding one, and the heat radiation from the walls of the pot as well as the gases evolved can only reach a comparatively small portion of each sheet inside of its edge, as indicated by shading 14 in Fig. 2, while the central portion of the sheet, which in the drawing is left blank, indicated the region which is not sensibly affected by heat radiation from the wall of the pot or by the gases evolved. This represents the effect of the old conventional annealing practice.

The object of annealing magnetic material, and especially silicon steel material, is to improve its magnetic characteristics, its hysteresis and permeability, and it will be seen that when the sheets upon which the effect of the old process is indicated in Fig. 110

2 are cut into shapes suitable for transformer cores or other magnetic cores, some portion of these cut pieces will be well annealed while others will be poorly or barely 5 annealed; and the irregularity of the distribution of the well and poorly annealed portions is in consequence such that no two cores built up of such material will have the same magnetic characteristics. In the annealing pots there is usually a series of holes 10 all along the walls of the same, whereby the gases developed inside the pot are allowed to circulate both within the pot and also between the pot and the furnace. This 15 has been found to be of considerable advantage. But the circulation which these holes would afford can only benefit a small and irregular portion of each sheet, as indicated in Fig. 2 by the shading 14.

20 In accordance with my invention the arrangement shown in Fig. 3 may be used. The annealing pot is the same as in Fig. 2, but the arrangement of the sheets within the pot differs from the old practice. Here the 25 mass of the sheets is shown to be divided into small bundles 16, each bundle comprising a limited number of sheets, placed face to face and loosely held together by a number of clips 17, of band iron. These clips 30 are liberally spaced and they do not forcibly press the sheets together, but they prevent the shifting of the sheets and make of each bundle a unit, the elements of which, the single sheets, are in loose contact and still 35 sufficiently separated by sensible spaces through which the heat radiation and the evolved gases can pass. Each of these bundles 16, is arranged vertically in the pot, with its lower edge raised from the floor of 40 the pot by the thickness of the clips 17, and the successive bundles are spaced from each other by the same clips. The lower edge of each bundle has only to sustain its own weight and no bundle presses upon another, 45 so that the small spaces between the individual sheets are maintained and each bundle is laterally braced by the others. With the arrangement shown in Fig. 3, the conditions 50 of the individual sheets as respects the access to the same of heat radiation and circulation of the evolved gases and of the gases which enter the pot by the vent holes 15 is largely promoted, and is practically the same as if the sheets, standing on edge, were 55 all loosely held together by any kind of lateral props. There is, however, this important practical difference between the two arrangements, that, the division of the whole charge of a pot into bundles, in accordance 60 with my invention, renders the procedure fit

for extensive and uniform commercial practice, whereas the arrangement of the whole charge in one mass of a multitude of loose sheets, is difficult and vexatious, and allows each sheet to buckle and have its lower edge 65 bent.

Another practical manner of realizing my invention is shown in Fig. 4. In this case the sheets are piled up flatwise in the pots, so as to form a stack, but the mass is subdivided into sections 16', each section comprising a limited number of sheets, about the same as the bundles 16 of Figs. 3 and 5; they are, however, in this case not necessarily held together by clips, but each section 70 is spaced from the next succeeding or preceding section by strips 17' of band iron, so that each section as a whole is free to the access of heat radiation and to the circulation of evolved gases, and of the gases 80 which enter by the vent holes 15 while each individual sheet is held to the next preceding one by light pressure at the separating strips and there is barely any pressure between the successive strips. I have found 85 by continued commercial use of this arrangement that the sheets become well annealed all over, so that this form of my invention is as effective as the arrangement shown in Fig. 3, or as the arrangement heretofore referred to, where the whole charge is put into the pot edgewise in one lot of a multitude of loose sheets.

What I claim as new and desire to secure by Letters Patent of the United States, is:— 95

1. The process of annealing a mass of sheets of magnetic material, which consists in dividing the mass into bundles or sections of a limited number of loosely contacting sheets, assembling the bundles or sections in an annealing pot in such manner so as to leave the faces of the sheets and of the bundles or sections free to the access of radiant heat and to the sweep of gases evolved in the pot and outside of the same, and subjecting the assembled bundles or sections to a suitable annealing temperature. 100

2. The process of annealing a mass of sheets of magnetic material, which consists in dividing the mass into loose sections or 110 bundles of a limited number of sheets, piling the sections or bundles flatwise in an annealing pot with sensible spaces between the same, and promoting the sweep of internally and externally evolved gases over the bundles and sheets while subjecting the whole to a suitable annealing temperature. 115

In witness whereof I have hereunto set my hand this 14th day of December, 1918.

WILLIAM J. WOOLDRIDGE.